# EUROPEAN PATENT SPECIFICATION

(11) **EP 1 866 261 B1**
(45) Date of publication and mention of the grant of the patent: **27.08.2008**
(21) Application number: 05807609.2
(22) Date of filing: 16.11.2005
(51) Int. Cl.: C04B 35/76, C04B 35/80, B32B 18/00, E04B 1/20

(54) **IMPROVED CERAMIC SLAB FOR FACINGS, AND METHOD FOR ITS MANUFACTURE**
VERBESSERTE KERAMIKPLATTE FÜR VERKLEIDUNGEN UND HERSTELLUNGSVERFAHREN DAFÜR
DALLE DE CERAMIQUE AMELIOREE POUR PAREMENTS, ET PROCEDE DE FABRICATION DE CELLE-CI

(30) Priority: 24.03.2005 IT RE20050030
(43) Date of publication of application: 19.12.2007
(73) Proprietor: SACMI COOPERATIVA MECCANICI IMOLA SOCIETA' COOPERATIVA, 40026 Imola (Bologna) (IT)
(72) Inventor: VALLI, Silvano, I-40027 Mordano (IT); RICCI, Claudio, I-40026 Imola (IT)
(74) Representative: Corradini, Corrado
(86) International application number: PCT/EP2005/012364
(87) International publication number: WO 2006/099894

(56) References cited:
- EP-A- 0 024 360
- EP-A- 0 737 787
- EP-A- 1 594 666
- WO-A-20/04022295
- BE-A1- 896 126
- DE-A1- 4 002 601
- GB-A- 1 536 663
- PATENT ABSTRACTS OF JAPAN vol. 1999, no. 09, 30 July 1999 (1999-07-30) & JP 11 100939 A (YOSHIKAWA KAIJI KOGYO KK), 13 April 1999 (1999-04-13)
- PATENT ABSTRACTS OF JAPAN vol. 018, no. 265 (M-1608), 20 May 1994 (1994-05-20) & JP 06 042063 A (MIE ASANO CONCRETE KK; others: 01), 15 February 1994 (1994-02-15)

## Description

### TECHNICAL FIELD

The present invention relates generally to ceramic slabs or tiles for facings and floorings, and to a method for their manufacture.

### BACKGROUND ART

Ceramic slabs usually used for facings and floorings are known to present high compression resistance, surface hardness and abrasion resistance characteristics, which are provided by the constituent materials of the ceramic mix and the high temperature firing process to which the mix is subjected.

In contrast, said ceramic slabs present low tensile strength and generally a fragile behaviour, which has always limited their use under conditions in which a state of tensile or bending stress is present.

Under such conditions, as the result of a knock or a particularly intense stress, a small crack can form within the ceramic slab, and because of the fragile ceramic behaviour can propagate progressively throughout the entire slab, until it breaks.

This intrinsic ceramic fragility is particularly serious if said slabs are used for facing external facades of buildings, as they may be fixed, generally by suitable mechanical means, at a great height from the ground.

In this context, there is an obvious danger arising from a sudden breakage of the slab (due to natural or accidental events) and the consequent fall of its fragments from a great height.

To confront this problem, two possible alternative solutions are currently known.

A widely used first solution consists of applying a net of synthetic or metallic material to the rear face of the ceramic slab by gluing with epoxy resin.

In this manner, if the slab suddenly breaks, its fragments remain in position retained by the net to which they are glued, so preventing danger to persons or things.

A recently introduced second solution consists of producing the slab by superposing two or more thin slabs and interposing a resin layer therebetween, which by gluing them together provides mechanical continuity to the assembly. In this manner a composite ceramic slab is obtained, in which each individual constituent slab acts as a support for the others.

Notwithstanding the good results offered by both said solutions, they present serious limitations to their widespread use, in particular because of the lack of reliability of the glue connection and the high cost of making this type of connection.

An object of the present invention is to provide a reinforced ceramic slab presenting resistance characteristics superior to usual slabs, within the framework of a simple, rational and low-cost solution.

### DISCLOSURE OF THE INVENTION

This object is attained by a reinforced ceramic slab comprising a continuous ceramic matrix internally incorporating reinforcement fibres, i.e. filiform bodies not necessarily rectilinear, having resistance characteristics superior to those of the ceramic matrix itself.

In particular, the reinforcement fibres possess greater tensile strength than said ceramic matrix.

The document JP 11 100939 discloses a reinforced concrete slab comprising a net reinforcing fibres positioned and tensed within the slab.

The fibres are distributed in alignments or strips forming a lattice and are not separated one another.

An epoxy resin is applied to the fibres to solidify and form fiber strips, and the intersections of the strips are tied.

According to the invention, the reinforcement fibres are distributed within said ceramic matrix in such a manner as to form at least one composite layer of ceramic and fibres lying between two purely ceramic layers.

Within said composite layer, the reinforcement fibres lie separated and spaced apart from each other substantially in one and the same plane, which can be parallel to the faces of the ceramic slab or inclined to them.

In particular, the reinforcement fibres can be distributed as to lie separately and spaced apart in random manner, or preferably can be distributed in an ordered manner to form a discontinuous net, the meshes of which are defined by the reinforcement fibres.

By virtue of this solution, a ceramic slab according to the invention is substantially provided with an inner reinforcement, which makes it less fragile than the usual completely ceramic slabs.

In this respect, if a crack forms within the reinforced ceramic slab, its propagation is interrupted on encountering the reinforcement fibres, which have greater resistance than the ceramic matrix, and which hence prevent the slab from breaking into fragments.

According to the invention, the meshes of the net must have their sides of length less than the length of the reinforcement fibres which define them, to prevent substantially rectilinear preferential directions existing within the ceramic slab along which a crack can propagate without encountering any reinforcement fibre.

In a preferred embodiment of the invention, the reinforcement fibres are distributed in an ordered repetitive pattern, so that the meshes of the discontinuous net are in the form of a parallelogram, typically rectangular or square, and are all equal to each other.

Furthermore, according to the invention, the reinforcement fibres are metal fibres, typically rectilinear pieces of steel wire, preferably having a diameter between 0.3 and 0.7 mm, and a length between 20 and 200 mm, preferably between 40 and 100 mm.

Alternatively, said reinforcement fibres can be glass fibres, carbon fibres or aramid fibres.

The invention also comprises a method for manufacturing said reinforced ceramic slab, comprising the following steps:
a) creating, on a support surface, a first layer of ceramic powder;
b) distributing an assembly of reinforcement fibres over at least an area of the top surface of said first layer of powder;
c) covering the reinforcement fibres, to create at least a second layer of ceramic powder on said first layer, in order to obtain a soft ceramic blank of desired thickness, containing the reinforcement fibres;
d) pressing said soft blank to compact the powders and obtain an unfired ceramic slab; and finally
e) subjecting said unfired ceramic slab to firing, to obtain a reinforced slab comprising a continuous ceramic matrix within which the reinforcement fibres are incorporated.

According to the invention, in particular, said step c) of covering the reinforcement fibres can be implemented by repeating steps a) and b) a desired number of times, so that the soft blank comprises a plurality of ceramic powder layers, between which the reinforcement fibres are interposed.

With this solution, the reinforced ceramic slab can be manufactured very simply, rationally and economically, both by a discontinuous forming process using usual ceramic moulds, and by a continuous forming process, of the type described in European patent application EP 1283097 in the name of the same Applicant.

In the first case, said support surface is a vertically translating surface, defined by the upper surface of the lower die of a ceramic mould, whereas in the second case it is a horizontally translating surface, defined by the conveyor belt of a continuous forming plant.

According to the invention, the reinforcement fibres are distributed over the entire top surface of the first layer of ceramic powder created, this preferably being a flat surface which can be parallel to the support surface or inclined to it.

The reinforcement fibres are distributed separated and spaced apart over said top surface in such a manner as to reduce to a minimum the region of ceramic mass within which possible cracks can propagate.

In particular, said reinforcement fibres can be distributed in random manner, but they are preferably distributed in an ordered manner to form a discontinuous net, the meshes of which are defined by the reinforcement fibres themselves; said meshes preferably having sides of dimensions less than the length of the fibres which define them.

In this manner, by using separate and easily applied reinforcement fibres, the method of the invention can be easily adapted to changes in ceramic slab format.

Moreover, said reinforced fibres advantageously enable natural linear expansion of the ceramic mass immediately after the pressing step, and its shrinkage during firing, during which in particular, notwithstanding the high temperatures, the reinforced fibres (especially those of metal or carbon) maintain their mechanical properties unaltered, they being embedded in the ceramic mass and not in contact with the oxygen of the air.

According to a preferred embodiment of the invention, the reinforced fibres are distributed as a plurality of longitudinal parallel rows and as a plurality of transverse parallel rows which intersect to form said discontinuous net, this hence presenting meshes of parallelogram shape. Moreover, the reinforced fibres of each longitudinal row are preferably offset from those pertaining to the adjacent longitudinal rows, the reinforced fibres of each transverse row likewise being offset from those pertaining to the adjacent transverse rows, so that the net meshes can have any desired dimension without involving superposing and mutual contact of the reinforced fibres.

According to a preferred embodiment, the distance separating the longitudinal rows and the distance separating the transverse rows are both constant and are preferably equal, to hence obtain a discontinuous net with its meshes all identical.

According to a further preferred embodiment of the invention, said longitudinal and transverse rows are inclined to the sides of the ceramic slab, preferably at an angle of about 45°.

By virtue of this embodiment, if the slab is subjected to a cutting step, for example after the pressing step, the cutting lines, which are generally parallel to the sides of the slab, intersect the reinforced fibres only within a limited region, to ensure good finishing of the resultant edge, and avoiding ceramic slab stability problems.

### BRIEF DESCRIPTION OF THE DRAWINGS

Further characteristics and advantages of the invention will become apparent on reading the ensuing description provided by way of nonlimiting example, with the aid of the figures shown in the accompanying drawings, in which:
Figure 1 is a partially cut-away view of a reinforced ceramic slab according to the invention;
Figure 2 is a side view of the slab of Figure 1;
Figures 3a to 3c show schematically a succession of steps in the method for manufacturing the slab of Figure 1;
Figure 4 is a plan view of Figure 3b;
Figure 4' is the same as Figure 4 but showing an alternative embodiment of the slab of Figure 1;
Figure 5 is a side view of a continuous plant for forming reinforced ceramic slabs according to the invention;
Figure 6 is a plan view of the forming plant shown in Figure 5;
Figures 7a to 7d show a ceramic mould during a succession of steps in the discontinuous forming process for the slab of Figure 1;
Figure 8 is an enlarged detail of Figure 5.

### BEST MODE FOR CARRYING OUT THE INVENTION

The reinforced ceramic slab 1, shown in Figure 1, comprises a continuous ceramic matrix 2, within which reinforcement fibres 3 are incorporated.

In the particular illustrated example, said reinforced fibres are rectilinear pieces of steel wire, preferably stainless steel; however, in general they can be filiform bodies, not necessarily rectilinear, of a material having resistance characteristics superior to those of the ceramic matrix 2, for example carbon fibres, glass fibres or aramid fibres.

As shown in Figure 1, the reinforced fibres 3 are distributed in the interior of the ceramic matrix in such a manner as to define a composite layer 20 of ceramic and fibres lying between two purely ceramic layers 20 and 21 (see also Figure 2), within said layer the reinforced fibres 3 lying substantially on one and the same surface, separated and spaced apart, to form a discontinuous net.

In this manner, whenever a crack forms in the ceramic slab 1, its propagation is interrupted on encountering the reinforced fibres 3, which have greater tensile strength than the ceramic matrix 2, and hence prevent the ceramic slab 1 from breaking into fragments.

As shown in the particular example of Figure 1, the reinforced fibres 3 are all of the same length, preferably between 40 mm and 100 mm, and the same diameter, preferably between 0.3 mm and 0.7 mm; in addition, the meshes of the discontinuous net, which are defined by the reinforced fibres 3, are substantially square.

The side dimension of said meshes is less than the length of the reinforced fibres 3, so that no substantially rectilinear preferential directions exist along which a crack can propagate without encountering any reinforced fibre 3.

A preferred method for manufacturing reinforced ceramic slabs 1 of the aforedescribed type is described hereinafter with the aid of Figures 3a-3c. Said manufacturing method comprises the following steps:
- creating, on a support surface 11, a first layer 5 of ceramic powders having a thickness substantially one half of the thickness of the soft ceramic mass which is to form the slab 1 (see Figure 3a);
- distributing an assembly of reinforcement fibres (3) over the top surface 50 of said first layer 5 (see Figure 3b);
- covering said reinforcement fibres 3, to create a second layer 6 of ceramic powders on said first layer 5, in order to obtain a soft ceramic blank containing the reinforcement fibres 3;
- pressing said soft blank to compact the powders and obtain an unfired ceramic slab; and finally
- subjecting said unfired ceramic slab to firing, to obtain a slab 1 comprising a continuous ceramic matrix 2 with the reinforcement fibres 3 incorporated in its interior.

As shown in Figure 4, said manufacturing method comprises distributing the reinforced fibres 3 over the surface 50 of the first layer 5 in an ordered manner, separated and spaced from each other, to form said discontinuous net.

In detail, the reinforced fibres 3 are aligned along a plurality of longitudinal parallel lines 30 and along a plurality of transverse parallel lines 31 parallel to the former.

The reinforced fibres 3 of each longitudinal row 30 are offset from the fibres 3 pertaining to the adjacent rows 30, and likewise the fibres 3 of each transverse row 31 are offset from those pertaining to the adjacent rows 31.

Moreover, the distance P between the longitudinal rows 30 and the distance P' between the transverse rows 31 are both constant, equal to each other and less than the length of the individual reinforced fibres 3, to obtain a discontinuous net with square meshes, all equal, having the length of their side less than said length of the reinforced fibres 3.

In the particular example shown in Figure 4, the longitudinal rows 30 and the transverse rows 31 are parallel respectively to the edges of the first ceramic layer 5, and hence to the edges of the reinforced slab 1 being manufactured. However, these rows 30 and 31 can also be inclined to the edges of the slab 1 and in particular, as shown in Figure 4', can be inclined by an angle substantially of 45°, for the reasons which will become clear hereinafter.

According to a first preferred embodiment of the method, shown in Figures 5 and 6, the reinforced ceramic slabs 1 are manufactured by a continuous forming plant 8.

Said forming plant 8 comprises schematically: a conveyor belt 80; first ceramic powder dispensing means 81; a distributor device 82 for reinforced fibres 3; second ceramic powder dispensing means 83; continuous powder compacting means 84; and finally cutting means 85 downstream of said compacting means 84.

In use, the first dispensing means 81 are arranged to deposit a first continuous layer of ceramic powder onto the upper surface 11 of the advancing belt 80; the distributor device 82, which is positioned downstream of the means 81, then distributes the reinforced fibres 3, which are all identical, over the top surface 50 of the first powder layer 5, in such a manner as to form the discontinuous net in accordance with the aforedescribed modality.

In particular, as visible in Figure 8, the longitudinal rows 30 and the transverse rows 31 are inclined to the sides of the first ceramic powder layer 5 by an angle substantially equal to 45°.

Downstream of the distributor device 82, the second dispensing means 83 deposit a second continuous layer 6 of ceramic powder onto the surface 50 of the first layer 5, to cover the reinforced fibres 3; said second layer 6 being able to present graphic effects within the powder mass or on its top surface.

In this manner, a continuous strip 7 of ceramic powder containing the reinforced fibres 3 is formed, and is made to advance on the conveyor belt 80 between the compacting means 84, which subject the ceramic powders to pressing to form a compact strip 7'. Said compacting means 84 are described in European patent application EP 1283097, to which reference should be made for further details.

Finally, the compact strip 7' is fed to the cutting means 85, which trim its edge and divide it into an assembly of separate unfired slabs 9.

In particular, as shown in Figure 8, said step of dividing the strip 7' into unfired slabs 9 takes place along cutting lines A perpendicular to the sides of the strip 7'; consequently, because of the already described distribution of reinforced fibres 3 along longitudinal lines 30 and transverse lines 31 inclined to the sides of the compact strip 7', said cutting lines A intersect the reinforced fibres 3 within limited regions, to obtain a good edge finish on the resultant unfired slab 9, without compromising its stability.

On termination of the cutting step, the unfired slabs 9 can finally be decorated, and may be subjected to a further pressing step using ceramic moulds, before being subjected to the traditional drying and firing steps, which enable the finished reinforced slab 1 to be obtained.

After the cutting step, the edges of the slab 1 may be smoothed and ground.

According to an alternative embodiment, shown in Figures 7a to 7d, the manufacture of the reinforced ceramic slabs 1 takes place by a discontinuous process using a usual ceramic mould 10.

Said mould 10 comprises a die plate 100 provided with a forming cavity 101, the base of which is closed by a lower movable die 102, with which an upper movable die 103 is vertically aligned.

A usual movable loading tray (not shown) can be associated with the mould 10 to release powdered ceramic material into the interior of the forming cavity 101.

In use, the manufacturing cycle conventionally begins when the upper surface 11 of the lower die 102 of the mould 10 is coplanar with the top of the die plate 100.

At this point the loading tray advances to above the forming cavity 101; then, as shown in Figure 7a, the lower die 102 is lowered by an amount substantially equal to one half the thickness of the soft ceramic mass intended to form the slab 1, so that a first layer 5 of ceramic powder descends to fill the forming cavity 101, in contact with the surface 11 of the lower die 102.

After this step, the loading tray withdraws, and reinforced fibres 3 are distributed over the top surface 50 of the first layer 5 (see Figure 7b), in a manner similar to that described for the preceding embodiment.

At this point the loading tray again advances and, as shown in Figure 7c, the lower die 102 is again lowered, enabling a second layer 6 of ceramic powders to descend to cover the reinforced fibres 3.

Finally (see Figure 7d), the upper die 103 is lowered to compact the soft ceramic mass, and hence obtain an unfired slab 9 which can then be subjected to the usual accessory steps, such as decoration or trimming, before being subjected to drying and firing in a kiln.

## Claims

1. A reinforced ceramic slab, comprising a continuous ceramic matrix (2) internally incorporating reinforcement fibres (3) having greater tensile strength than the ceramic matrix (2) where said reinforced fibres (3) are distributed within the interior of the ceramic matrix (2) in such a manner as to form at least one composite layer (20) of ceramic and fibres, lying between two purely ceramic layers (21, 22), **characterised by** the fact that the reinforced fibres (3) are distributed as to lie separated and spaced apart.

2. A slab as claimed in claim 1, **characterised in that** within the composite layer (20), the reinforced fibres are distributed in such a manner as to lie substantially in the same plane, separated and spaced apart.

3. A slab as claimed in claim 2, **characterised in that** said plane is substantially parallel to the faces of the slab (1).

4. A slab as claimed in claim 2, **characterised in that** said plane is inclined to the faces of the slab (1).

5. A slab as claimed in claim 2., **characterised in that** the reinforced fibres (3) are distributed in a random manner.

6. A slab as claimed in claim 2, **characterised in that** the reinforced fibres (3) are distributed in an ordered manner to form a discontinuous net, the meshes of which are defined by the reinforced fibres (3).

7. A slab as claimed in claim 6, **characterised in that** the meshes of the net have sides of length less than the length of the reinforced fibres (3) which define them.

8. A slab as claimed in claim 6, **characterised in that** the meshes of the net are of parallelogram shape.

9. A slab as claimed in claim 8, **characterised in that** the meshes of the net are substantially all equal.

10. A slab as claimed in claim 1, **characterised in that** said reinforced fibres (3) are metal fibres.

11. A slab as claimed in claim 10, **characterised in that** said metal fibres (3) are rectilinear pieces of steel wire.

12. A slab as claimed in claim 11, **characterised in that** said steel wire pieces have a diameter between 0.3 mm and 0.7 mm.

13. A slab as claimed in claim 11, **characterised in that** the steel wire pieces have a length between 20 mm and 200 mm.

14. A slab as claimed in claim 13, **characterised in that** the steel wire pieces have a length between 40 mm and 100 mm.

15. A slab as claimed in claim 1, **characterised in that** said reinforced fibres (3) are chosen from the group comprising carbon fibres, aramid fibres and glass fibres.

16. A method for manufacturing reinforced ceramic slabs (1) in accordance with claim 1, **characterised by** comprising the following steps:
a) creating, on a support surface (11), a first layer of ceramic powder (5);
b) distributing an assembly of reinforcement fibres (3) over at least an area of the top surface (50) of said first layer (5) of ceramic powder;
c) covering the reinforcement fibres, to create at least a second layer (6) of ceramic powder on said first layer (5), in order to obtain a soft ceramic blank of desired thickness containing the reinforcement fibres;
d) pressing said soft blank to compact the powders and obtain an unfired ceramic slab;
e) subjecting said unfired ceramic slab to firing, to obtain a ceramic slab (1) comprising a continuous ceramic matrix (2) with the reinforcement fibres (3) incorporated.

17. A method as claimed in claim 16, **characterised in that** step c) is implemented by repeating steps a) and b), to obtain a soft blank comprising a plurality of ceramic powder layers between which the reinforced fibres (3) are interposed.

18. A method as claimed in claim 16, **characterised in that** the reinforced fibres (3) are distributed over the entire top surface (50) of the first ceramic powder layer (5).

19. A method as claimed in claim 16, **characterised in that** the top surface (50) of the first layer (5) is a flat surface.

20. A method as claimed in claim 19, **characterised in that** said top surface (50) is parallel to the support surface (11) on which the first ceramic powder layer (5) is created.

21. A method as claimed in claim 19, **characterised in that** said top surface (50) is inclined to the support surface (11).

22. A method as claimed in claim 16, **characterised in that** the reinforced fibres (3) of each assembly are distributed such that they are separated and spaced apart.

23. A method as claimed in claim 16, **characterised in that** the reinforced fibres (3) are distributed in a random manner.

24. A method as claimed in claim 16, **characterised in that** the reinforced fibres (3) are distributed in an ordered manner such as to form a discontinuous net, the meshes of which are defined by the reinforced fibres (3).

25. A method as claimed in claim 24, **characterised in that** the meshes of the discontinuous net have sides of length less than the length of the reinforced fibres (3) which define them.

26. A method as claimed in claim 24, **characterised in that** the reinforced fibres (3) are distributed as a plurality of longitudinal parallel rows (30) and a plurality of transverse parallel rows (31) oblique to the longitudinal rows (30).

27. A method as claimed in claim 24, **characterised in that** the reinforced fibres (3) pertaining to each longitudinal row (30) are offset from those pertaining to the adjacent longitudinal rows (30), the reinforced fibres (3) pertaining to each transverse row (31) being offset from those pertaining to the adjacent transverse rows (31).

28. A method as claimed in claim 26, **characterised in that** said longitudinal rows (30) are spaced apart by a constant distance (P), the transverse rows (31) being likewise spaced apart by a constant distance (P').

29. A method as claimed in claim 28, **characterised in that** the distance (P) separating the longitudinal rows (30) is equal to the distance (P') separating the transverse rows (31).

30. A method as claimed in claim 26, **characterised in that** said longitudinal rows (30) and transverse rows (31) are inclined to the sides of the ceramic slab (1).

31. A method as claimed in claim 30, **characterised in that** said longitudinal rows (30) and transverse rows (31) are inclined substantially at 45° to the sides of the ceramic slab (1).

32. A method as claimed in claim 16, **characterised in that** the support surface (11) on which the first ceramic powder layer (5) is created is a translating surface.

33. A method as claimed in claim 32, **characterised in that** said support surface (11) translates in a vertical direction.

34. A method as claimed in claim 32, **characterised in that** said support surface (11) translates in a horizontal direction.

35. A method as claimed in claim 33, **characterised in that** said support surface (11) is defined by the upper surface of the lower die (102) of a ceramic mould (10).

36. A method as claimed in claim 34, **characterised in that** said support surface (11) is defined by the conveyor belt (80) of a continuous pressing plant.

37. A method as claimed in claim 16, **characterised in that** step c) is followed by a step of decorating the unfired slab.

38. A method as claimed in claim 16, **characterised in that** step c) is followed by a second pressing of the unfired slab.

39. A method as claimed in claim 16, **characterised in that** step c) is followed by a step of cutting the unfired ceramic slab.

40. A method as claimed in claim 16, **characterised in that** step d) is followed by a step of smoothing and grinding the edges of the ceramic slab (1).

## Patentansprüche

1. Eine faserverstärkte Keramik-Platte, einschließlich einer fortlaufenden Keramikmatrix (2), innen ausgestattet mit Verstärkungsfasern (3) mit höherer Zerreißfestigkeit als die Keramikmatrix (2), wobei die Verstärkungsfasern (3) im Inneren der Keramikmatrix (2) so verteilt sind, dass zwischen zwei reinen Keramiklagen (21, 22) wenigstens eine aus Keramik und Fasern geformte Verbundlage (20) liegt, **dadurch gekennzeichnet, dass** die Verstärkungsfasern (3) so verteilt sind, dass sie einzeln und mit Zwischenräumen zueinander liegen.

2. Eine Platte nach Anspruch 1, **dadurch gekennzeichnet, dass** in der Verbundlage (20) die Verstärkungsfasern so verteilt sind, dass sie im Wesentlichen einzeln und mit Zwischenräumen zueinander auf einer selben Ebene liegen.

3. Eine Platte nach Anspruch 2, **dadurch gekennzeichnet, dass** die Ebene im Wesentlichen parallel zu den Flächen der Platte (1) liegt.

4. Eine Platte nach Anspruch 2, **dadurch gekennzeichnet, dass** die Ebene schräg zu den Flächen der Platte (1) liegt.

5. Eine Platte nach Anspruch 2, **dadurch gekennzeichnet, dass** die Verstärkungsfasern (3) zufällig verteilt sind.

6. Eine Platte nach Anspruch 2, **dadurch gekennzeichnet, dass** die Verstärkungsfasern (3) so angeordnet sind, dass sie ein diskontinuierliches Netz formen, dessen Maschen von den Verstärkungsfasern (3) gebildet werden.

7. Eine Platte nach Anspruch 6, **dadurch gekennzeichnet, dass** die Maschen des Netzes eine geringere Seitenlänge als die Länge der Verstärkungsfasern (3) haben, aus denen sie gebildet werden.

8. Eine Platte nach Anspruch 6, **dadurch gekennzeichnet, dass** die Maschen des Netzes die Form eines Parallelogramms haben.

9. Eine Platte nach Anspruch 8, **dadurch gekennzeichnet, dass** die Netzmaschen im Wesentlichen alle gleich sind.

10. Eine Platte nach Anspruch 1, **dadurch gekennzeichnet, dass** die Verstärkungsfasern (3) aus Metall sind.

11. Eine Platte nach Anspruch 10, **dadurch gekennzeichnet, dass** die Metallfasern (3) geradlinige Stücke aus Stahldraht sind.

12. Eine Platte nach Anspruch 11, **dadurch gekennzeichnet, dass** die Stahldrahtstücke einen Durchmesser zwischen 0,3 mm und 0,7 mm haben.

13. Eine Platte nach Anspruch 11, **dadurch gekennzeichnet, dass** die Stahldrahtstücke eine Länge zwischen 20 mm und 200 mm haben.

14. Eine Platte nach Anspruch 13, **dadurch gekennzeichnet, dass** die Stahldrahtstücke eine Länge zwischen 40 mm und 100 mm haben.

15. Eine Platte nach Anspruch 1, **dadurch gekennzeichnet, dass** die Verstärkungsfasern (3) aus einer Gruppe aus Kohlefasern, Aramidfasern und Glasfasern ausgewählt werden.

16. Ein Verfahren zur Herstellung verstärkter Keramikplatten (1) nach Anspruch 1, **gekennzeichnet durch** die folgenden Schritte:
a) Erzeugen einer ersten Lage Keramikpulver (5) auf einer Auflagefläche (11);
b) Verteilen von Verstärkungsfasern (3) auf wenigstens einem Bereich der oben liegenden Fläche (50) der ersten Lage (5) aus Keramikpulver;
c) Bedecken der Verstärkungsfasern mit wenigstens einer zweiten Lage (6) Keramikpulver auf der ersten Lage (5), um einen weichen Keramikrohling der gewünschten Dicke mit eingebetteten Verstärkungsfasern zu erhalten;
d) Pressen des weichen Rohlings zum Verdichten des Pulvers und für Erhalt einer ungebrannten Keramikplatte;
e) Brennen der ungebrannten Keramikplatte, um eine Keramikplatte (1) aus einer fortlaufenden Keramikmatrix (2) mit eingebetteten Verstärkungsfasern (3) zu erhalten.

17. Ein Verfahren nach Anspruch 16, **dadurch gekennzeichnet, dass** Schritt c) durch die Wiederholung der Schritte a) und b) durchgeführt wird, um einen weichen Rohling aus einer Vielzahl an Keramikpulverlagen zu erhalten, zwischen denen die Verstärkungsfasern (3) angeordnet sind.

18. Ein Verfahren nach Anspruch 16, **dadurch gekennzeichnet, dass** die Verstärkungsfasern (3) über die gesamte oben liegende Fläche (50) der ersten Keramikpulverlage (5) angeordnet sind.

19. Ein Verfahren nach Anspruch 16, **dadurch gekennzeichnet, dass** die oben liegende Fläche (50) der ersten Lage (5) eine ebene Fläche ist.

20. Ein Verfahren nach Anspruch 19, **dadurch gekennzeichnet, dass** die oben liegende Fläche (50) parallel zur Auflagefläche (11) liegt, auf der die erste Keramikpulverlage (5) erzeugt wird.

21. Ein Verfahren nach Anspruch 19, **dadurch gekennzeichnet, dass** die oben liegende Fläche (50) schräg zur Auflagefläche (11) liegt.

22. Ein Verfahren nach Anspruch 16, **dadurch gekennzeichnet, dass** die Verstärkungsfasern (3) jeder Lage so angeordnet sind, dass sie einzeln und mit Zwischenräumen zueinander liegen.

23. Ein Verfahren nach Anspruch 16, **dadurch gekennzeichnet, dass** die Verstärkungsfasern (3) zufällig verteilt sind.

24. Ein Verfahren nach Anspruch 16, **dadurch gekennzeichnet, dass** die Verstärkungsfasern (3) so angeordnet sind, dass sie ein diskontinuierliches Netz bilden, dessen Maschen von den Verstärkungsfasern (3) gebildet werden.

25. Ein Verfahren nach Anspruch 24, **dadurch gekennzeichnet, dass** die Maschen des diskontinuierlichen Netzes eine geringere Seitenlänge haben, als die Länge der sie bildenden Verstärkungsfasern (3).

26. Ein Verfahren nach Anspruch 24, **dadurch gekennzeichnet, dass** die Verstärkungsfasern (3) als eine Vielzahl an längs verlaufenden, parallelen Reihen (30) und eine Vielzahl an quer verlaufenden, parallelen Reihen (31) schräg zu den längs verlaufenden Reihen (30) angeordnet sind.

27. Ein Verfahren nach Anspruch 24, **dadurch gekennzeichnet, dass** die Verstärkungsfasern (3) in jeder Längsreihe (30) zu denen aus den anliegenden Längsreihen (30) versetzt liegen und die Verstärkungsfasern (3) jeder Querreihe (31) zu denen aus den anliegenden Querreihen (31) versetzt liegen.

28. Ein Verfahren nach Anspruch 26, **dadurch gekennzeichnet, dass** die Längsreihen (30) in einem konstanten Abstand (P) zueinander stehen und die Querreihen (31) ebenfalls in konstantem Abstand (P') zueinander stehen.

29. Ein Verfahren nach Anspruch 28, **dadurch gekennzeichnet, dass** der Abstand (P) zwischen den Längsreihen (30) dem Abstand (P') zwischen den Querreihen (31) gleich ist.

30. Ein Verfahren nach Anspruch 26, **dadurch gekennzeichnet, dass** die Längsreihen (30) und Querreihen (31) schräg zu den Seiten der Keramikplatte (1) liegen.

31. Ein Verfahren nach Anspruch 30, **dadurch gekennzeichnet, dass** die Längsreihen (30) und die Querreihen (31) im Wesentlichen um 45° schräg zu den Seiten der Keramikplatte (1) liegen.

32. Ein Verfahren nach Anspruch 16, **dadurch gekennzeichnet, dass** die Auflagefläche (11), auf der die erste Lage Keramikpulver (5) erzeugt wird, eine Übertragungsoberfläche ist.

33. Ein Verfahren nach Anspruch 32, **dadurch gekennzeichnet, dass** die Auflagefläche (11) in senkrechter Richtung überträgt.

34. Ein Verfahren nach Anspruch 32, **dadurch gekennzeichnet, dass** die Auflagefläche (11) in waagerechter Richtung überträgt.

35. Ein Verfahren nach Anspruch 33, **dadurch gekennzeichnet, dass** die Auflagefläche (11) die obere Fläche der unteren Matrize (102) einer Keramikgießform (10) ist.

36. Ein Verfahren nach Anspruch 34, **dadurch gekennzeichnet, dass** die Auflagefläche (11) das Förderband (80) einer fortlaufenden Pressanlage ist.

37. Ein Verfahren nach Anspruch 16, **dadurch gekennzeichnet, dass** auf Schritt c) ein Schritt zum Dekorieren der ungebrannten Keramikplatte folgt.

38. Ein Verfahren nach Anspruch 16, **dadurch gekennzeichnet, dass** auf Schritt c) ein zweites Pressen der ungebrannten Platte folgt.

39. Ein Verfahren nach Anspruch 16, **dadurch gekennzeichnet, dass** auf Schritt c) ein Schritt zum Schneiden der ungebrannten Keramikplatte folgt.

40. Ein Verfahren nach Anspruch 16, **dadurch gekennzeichnet, dass** auf Schritt d) ein Schritt zum Glätten und Schleifen der Ränder der Keramikplatte (1) folgt.

## Revendications

1. Une dalle de céramique renforcée, comprenant une matrice céramique continue (2) comprenant à l'intérieur des fibres de renfort (3) ayant des caractéristiques de résistance à la tension supérieures à celles de la matrice céramique (2) où lesdites fibres de renfort (3) sont distribuées à l'intérieur de la matrice céramique (2) de manière à former au moins une couche composite (20) de céramique et de fibres, reposant entre deux couches de céramique pure (21, 22), **caractérisée par le fait que** les fibres de renfort (3) sont distribuées de manière à être séparées et espacées.

2. Une dalle selon la revendication 1, **caractérisée par le fait qu'**à l'intérieur de la couche composite (20), les fibres de renfort sont distribuées de manière à reposer substantiellement sur le même plan, séparées et espacées.

3. Une dalle selon la revendication 2, **caractérisée par le fait que** ledit plan est substantiellement parallèle aux faces de la dalle (1).

4. Une dalle selon la revendication 2, **caractérisée par le fait que** ledit plan est incliné par rapport aux faces de la dalle (1).

5. Une dalle selon la revendication 2, **caractérisée par le fait que** les fibres de renfort (3) sont distribuées de manière aléatoire.

6. Une dalle selon la revendication 2, **caractérisée par le fait que** les fibres de renfort (3) sont distribuées de manière ordonnée pour former un filet discontinu, dont les mailles sont définies par les fibres de renfort (3).

7. Une dalle selon la revendication 6, **caractérisée par le fait que** les mailles du filet ont des côtés d'une longueur inférieure à celle des fibres de renfort (3) qui les définissent.

8. Une dalle selon la revendication 6, **caractérisée par le fait que** les mailles du filet sont en forme de parallélogramme.

9. Une dalle selon la revendication 8, **caractérisée par le fait que** les mailles du filet sont substantiellement toutes égales.

10. Une dalle selon la revendication 1, **caractérisée par le fait que** lesdites fibres de renfort (3) sont des fibres métalliques.

11. Une dalle selon la revendication 10, **caractérisée par le fait que** lesdites fibres métalliques (3) sont des morceaux rectilignes de fil d'acier.

12. Une dalle selon la revendication 11, **caractérisée par le fait que** lesdits morceaux de fil d'acier possèdent un diamètre compris entre 0,3 mm et 0,7 mm.

13. Une dalle selon la revendication 11, **caractérisée par le fait que** les morceaux de fil d'acier possèdent une longueur comprise entre 20 mm et 200 mm.

14. Une dalle selon la revendication 13, **caractérisée par le fait que** les morceaux de fil d'acier possèdent une longueur comprise entre 40 mm et 100 mm.

15. Une dalle selon la revendication 1, **caractérisée par le fait que** lesdites fibres de renfort (3) sont choisies dans le groupe comprenant les fibres de carbone, les fibres aramides et les fibres de verre.

16. Une méthode pour la fabrication des dalles de céramique renforcée (1) selon la revendication 1, **caractérisée par** l'inclusion des étapes suivantes :
a) création, sur une surface de support (11), d'une première couche de poudre de céramique (5) ;
b) distribution d'un ensemble de fibres de renfort (3) sur au moins une zone de la surface supérieure (50) de ladite première couche (5) de poudre de céramique ;
c) couverture des fibres de renfort, pour créer au moins une deuxième couche (6) de poudre de céramique sur ladite première couche (5), afin d'obtenir une ébauche souple de l'épaisseur désirée contenant les fibres de renfort ;
d) pressage de ladite ébauche afin de compacter les poudres et d'obtenir une dalle céramique non cuite ;
e) soumission de ladite dalle céramique non cuite à une cuisson, pour obtenir une dalle de céramique (1) comprenant une matrice céramique continue (2) avec les fibres de renfort (3) incorporées.

17. Une méthode selon la revendication 16, **caractérisée par le fait que** l'étape c) est mise en oeuvre en répétant les étapes a) et b) afin d'obtenir une ébauche souple comprenant plusieurs couches de poudre de céramique entre lesquelles sont intercalées les fibres de renfort (3).

18. Une méthode selon la revendication 16, **caractérisée par le fait que** les fibres de renfort (3) sont distribuées sur toute la surface supérieure (50) de la première couche de poudre de céramique (5).

19. Une méthode selon la revendication 16, **caractérisée par le fait que** ladite surface supérieure (50) de la première couche (5) est une surface plane.

20. Une méthode selon la revendication 19, **caractérisée par le fait que** ladite surface supérieure (50) est parallèle à la surface de support (11) sur laquelle la première couche de poudre de céramique (5) est créée.

21. Une méthode selon la revendication 19, **caractérisée par le fait que** ladite surface supérieure (50) est inclinée par rapport à la surface de support (11).

22. Une méthode selon la revendication 16, **caractérisée par le fait que** les fibres de renfort (3) de chaque ensemble sont distribuées de manière à être séparées et espacées.

23. Une méthode selon la revendication 16, **caractérisée par le fait que** les fibres de renfort (3) sont distribuées de manière aléatoire.

24. Une méthode selon la revendication 16, **caractérisée par le fait que** les fibres de renfort (3) sont distribuées de manière ordonnée afin de former un filet discontinu, dont les mailles sont définies par les fibres de renfort (3).

25. Une méthode selon la revendication 24, **caractérisée par le fait que** les mailles du filet discontinu ont des côtés d'une longueur inférieure à celle des fibres de renfort (3) qui les définissent.

26. Une méthode selon la revendication 24, **caractérisée par le fait que** les fibres de renfort (3) sont distribuées comme une multitude de rangées longitudinales (30) parallèles et une multitude de rangées transversales (31) parallèles obliques aux rangées longitudinales (30).

27. Une méthode selon la revendication 24, **caractérisée par le fait que** les fibres de renfort (3) appartenant à chaque rangée longitudinale (30) sont décalées de celles appartenant aux rangées longitudinales (30) adjacentes, les fibres de renfort (3) appartenant à chaque rangée transversale (31) étant décalées de celles appartenant aux rangées transversales (31) adjacentes.

28. Une méthode selon la revendication 26, **caractérisée par le fait que** lesdites rangées longitudinales (30) sont espacées d'une distance constante (P), les rangées transversales (31) étant également espacées d'une distance constante (P').

29. Une méthode selon la revendication 28, **caractérisée par le fait que** la distance (P) séparant les rangées longitudinales (30) est égale à la distance (P') séparant les rangées transversales (31).

30. Une méthode selon la revendication 26, **caractérisée par le fait que** lesdites rangées longitudinales (30) et rangées transversales (31) sont inclinées par rapport aux côtés de la dalle de céramique (1).

31. Une méthode selon la revendication 30, **caractérisée par le fait que** lesdites rangées longitudinales (30) et rangées transversales (31) sont inclinées substantiellement à 45° par rapport aux côtés de la dalle de céramique (1).

32. Une méthode selon la revendication 16, **caractérisée par le fait que** la surface de support (11) sur laquelle est créée la première couche de poudre de céramique (5) est une surface en translation.

33. Une méthode selon la revendication 32, **caractérisée par le fait que** ladite surface de support (11) effectue une translation dans une direction verticale.

34. Une méthode selon la revendication 32, **caractérisée par le fait que** ladite surface de support (11) effectue une translation dans une direction horizontale.

35. Une méthode selon la revendication 33, **caractérisée par le fait que** ladite surface de support (11) est définie par la surface supérieure de la couche inférieure (102) d'un moule céramique (10).

36. Une méthode selon la revendication 34, **caractérisée par le fait que** ladite surface de support (11) est définie par la bande convoyeuse (80) d'une installation de pressage en continu.

37. Une méthode selon la revendication 16, **caractérisée par le fait que** l'étape c) est suivie par une étape de décoration de la dalle non cuite.

38. Une méthode selon la revendication 16, **caractérisée par le fait que** l'étape c) est suivie par un deuxième pressage de la dalle non cuite.

39. Une méthode selon la revendication 16, **caractérisée par le fait que** l'étape c) est suivie par une étape de découpe de la dalle de céramique non cuite.

40. Une méthode selon la revendication 16, **caractérisée par le fait que** l'étape d) est suivie par une étape de polissage et de meulage des bords de la dalle de céramique (1).
